

# UNITED STATES PATENT OFFICE.

WILLIAM E. DOUBLEDAY, OF NEW YORK, N. Y.

## PROCESS OF TREATING FUR.

SPECIFICATION forming part of Letters Patent No. 350,455, dated October 5, 1886.

Application filed March 2, 1886. Serial No. 193,788. (No specimens.)

*To all whom it may concern:*

Be it known that I, WILLIAM E. DOUBLEDAY, a citizen of the United States, residing at New York, in the county of New York and State of New York, have invented certain new and useful Improvements in Processes for Treating Fur, of which the following is a specification.

It is well known to furriers and other dealers in and manufacturers of fur articles that there is a large waste of material, particularly of cony and similar furs which have been dyed black and other colors, arising from the fact that it has hitherto been impracticable to use the small pieces of fur which are left after cutting the skins into the desired shape during the manufacture of muffs, capes, cloaks, and various other manufactured articles.

The object of this invention is to utilize the fur upon such clippings and other pieces of skin as may from any cause become practically valueless for manufacture into garments or other articles; and to this end the invention consists in removing the fur from the skin and reducing it to a proper condition for subsequent treatment by felting or other manipulation, whereby it can be manufactured into articles—such as, for instance, hats—into which it enters either as the sole material, or in connection with other feltable or non-feltable fibers.

To this end I propose to treat the skin and attached fur by means of a suitable bath, hot or cold water, composed in whole or in part of an acid or an alkali, which will remove the color or change the color to such extent that it shall be unobjectionable. I propose, also, by means of this bath to so destroy, weaken, or modify the structure or texture and condition of the skin as to facilitate the next operation, which consists in subjecting the skin and attached fur fibers to the action of a "devil" or similar machine, whereby the skin is reduced to small fragments and the fur is detached therefrom. The tenacity with which the fur fibers originally adhered to the skin will be so reduced by the treatment in the bath that the fibers will not be injured by the operation of the devil or other separating-machine, or at least will not be injured to such an extent as to interfere seriously with their availability or value for use in subsequent manufacture.

I do not wish to be limited to the employment of any particular ingredients in the bath above referred to, but propose to use any of the well-known acid or alkali, or compounds of acids or alkali, with other ingredients which will properly effect the bleaching or change of color, and will at the same time so soften, rot, or disintegrate, or otherwise modify the condition of the skin that the fur fibers can be removed therefrom without serious injury; nor do I wish to be limited to the employment of a devil for separating the fur fibers from the skin, because I may substitute therefor any of the various well-known pickers which may be found adapted for that purpose; or, under some circumstances, I propose to subject the material to the action of crushing or reducing rollers after it has been removed from the bath and before it is subjected to the action of the devil or picker.

My experience proves the possibility of separating the skin and fur from each other by simply boiling the same in water, and afterward pouring off the water and the skin which is held in solution, together with such coloring-matter as has been extracted from the fur by the process of boiling.

The fur, after drying, will be found in suitable condition for the picker or other similar machine, whether it is desired to mix it with other material before use or to use it separately.

I further propose to subject the mass, after the bath, to "pot-carrotting," so called, when it will frequently be found that the product will be in proper condition for being either mixed with other material—such as wool or other fiber—or for being fed to an ordinary picker, blower, or other machinery for forming a bat or a hat.

What I claim is—

1. As an improvement in the art of treating fur, first subjecting the skin and adhering fur fibers to the action of a bath, and subsequently detaching the fur fibers from the skin, substantially as set forth.

2. As an improvement in the art of treating fur, first subjecting the skin and adhering fur fibers to the action of a bath, which changes the color of the fur fibers and changes the texture of the skin, and subsequently subjecting the material to the action of a machine, which

further reduces the skin to small fragments and detaches the fur fibers therefrom, substantially as set forth.

3. The process of removing the skin from the fur by subjecting them to the action of hot water, and then separating the water, with skin in solution, from the fur, substantially as set forth.

In testimony whereof I affix my signature in presence of two witnesses.

WILLIAM E. DOUBLEDAY.

Witnesses:

JAMES C. BALDWIN,  
GEO. GREGORY.